

# UNITED STATES PATENT OFFICE

2,118,686

## ALUMINUM ALLOY

Hans Steudel and Heinz Wiechell, Dessau, Germany, assignors to Junkers Flugzeug-und-Motorenwerke Aktiengesellschaft, Dessau, Germany

No Drawing. Application March 28, 1935, Serial No. 13,435. Renewed April 22, 1938. In Germany November 22, 1934

### 1 Claim. (Cl. 75—141)

Our invention relates to light metal alloys and more especially to an aluminum alloy containing, besides aluminum, copper and zinc as alloying metals. It is an object of our invention 5 to provide an alloy of this type, which is superior to similar alloys as far as hardness, strength and elongation are concerned.

We have found that an alloy containing, besides aluminum, copper and zinc, also iron, possesses particularly valuable properties and that alloys containing, besides aluminum, 1 to 12 per cent copper, 1 to 12 per cent zinc and 2.0 to 10 per cent iron are distinguished by great hardness 10 and strength and possess an elongation which is remarkable for a casting alloy.

As is known to those skilled in the art, aluminum alloys containing zinc show as a rule a comparatively great diminution of strength at increasing temperature. In the alloy according to 15 the present invention this drawback is removed by the addition of iron.

The new alloy is particularly suitable for use as a material for the manufacture of parts of machinery subject to sliding motion, such as 20 bearing bushings, guides, pistons etc.

We have found that the new alloy will possess particularly good sliding properties, if the copper and zinc are combined therein in substantially equal proportions. Thus for instances an alloy 25 containing, besides aluminum, about 8 per cent copper, 8 per cent zinc and 6 per cent iron, has done excellent services as a material for bushings and guides.

Another alloy containing, besides aluminum, about 2 per cent copper, 1 per cent zinc and 9 per cent iron, owing to the lower percentage of copper, is softer than the alloy first mentioned and possesses particularly good running properties. 5

The term "aluminum" as used in the present specification and claim includes not only pure aluminum but also commercial grades of aluminum containing the usual impurities or small amounts of other impurities insufficient in amount to alter the characteristic properties of the metal. 10

Various changes may be made in the details disclosed in the foregoing specification without departing from the invention or sacrificing the advantages thereof. 15

In the claim affixed to this specification no selection of any particular modification of the invention is intended to the exclusion of other modifications thereof and the right to subsequently make claim in the present application to any modification not covered by the claim is expressly reserved. 20

We claim:—

An aluminum alloy consisting of about 8 per cent copper, 8 per cent zinc and 6 per cent iron, with a remainder aluminum, said alloy being distinguished by great hardness and strength and possessing an elongation which is remarkable for 25 a casting alloy.

HANS STEUDEL.  
HEINZ WIECHELL.